

## UNITED STATES PATENT OFFICE.

GEORG ISING AND HEINRICH BOROFSKI, OF BRUNSWICK, GERMANY, ASSIGNEES, BY  
MESNE ASSIGNMENTS, TO THE CHEMICAL FOUNDATION, INC., A CORPORATION OF  
DELAWARE.

## PROCESS OF PRODUCING METAL BODIES.

No drawing.

Application filed October 31, 1918. Serial No. 260,609.

*To all whom it may concern:*

Be it known that we, GEORG ISING and HEINRICH BOROFSKI, citizens of the German Republic, residing at Brunswick, Adolf- 5 strasse 33, Germany, have invented certain new and useful Improvements in a Process of Producing Metal Bodies, of which the following is a specification.

Our invention relates to the art of producing metallic bodies and especially to the art of producing compound bodies of metals and admixtures. The object of our invention is to provide an improved process of uniting metals with metals, or with admixtures having 10 physical properties; that is, melting point, specific gravity, and so on, which are diverse from the corresponding physical properties of the particular metal with which the metal or the admixture is to be compounded. Hitherto, it was impossible, for instance, to produce by a fusing and casting action a metallic composition from aluminium and graphite powder in which the graphite particles would be uniformly 15 embedded within the preponderating primary metal without, incidentally, materially reducing the co-efficient of strength of the metal forming the base of the compound. Our present invention enables us 20 to intimately unite substances of diverse nature and physical properties. The union obtained is equivalent to a welded compound body that is free from defects, and the added substances are uniformly distributed 25 within the metallic constituent of the compound. To prevent a reduction of the strength of the compound body produced on account of the presence of oxides of the 30 primary metal constituent, we deoxidize the latter. The deoxidation may be carried out either prior to or during the process of uniting the different constituents of the compound body.

40 In accordance with our invention we are able to manufacture metals containing graphite which have a low co-efficient of friction. Such compounds may be employed, instead of the expensive bronze, for 45 guide bands on projectiles, for bearings, and for like purposes. In the same manner we may join hard substances to the metals whereby a compound having a high co- 50 efficient of friction is produced, such for

instance, as is required for grinding or 55 braking purposes.

Our invention comprises transforming the metal to be subjected to the pressure into a state of plasticity by means of heat or high pressure, or a combination of heat and 60 pressure, deoxidizing the metal and pressing the same into the desired shape. The deoxidation may precede the said transformation of the metal into a plastic state or may be carried out simultaneously with 65 said transformation. Another feature of our invention consists in adding another metal, or a non-metallic substance, to the primary metal while the latter is in a pulp-like or dough-like state, i. e., the said state 70 of plasticity, and then subjecting the mixture to pressure, whereby the added substance is permanently and firmly embedded within the primary metal and evenly distributed therein. 75

In order to render our invention more clear, we will now specifically describe, by means of examples, and for purposes of illustration only, the manner in which we may proceed to carry our invention into 80 effect.

I. The primary metal is reduced to a more or less plastic mass by means of heat or pressure and then deoxidized. The deoxidation may, for instance, consist in the 85 removal of the oxide film, whereupon we prevent the formation of a new oxide layer by providing a covering layer of carbonic acid gas or the like gaseous agent. Upon cooling the primary metal mass and simultaneously stirring into the same the substance to be added thereto we obtain the mass of the pulpy or dough-like state which we call the state of plasticity. While this state prevails pressure is applied, for instance, hydraulically, whereby the metallic particles are pressed together and, simultaneously, around the particles of the substance added. 90

II. We disintegrate the primary metal and 100 the substance to be added thereto, and mix these constituents of the compound to be produced. We then deoxidize the particles of the primary metal, for instance, by means of an acid or the like substance capable of a deoxidizing action. The thus treated mixture is transformed into a dough-like mass by heat, and then subjected 105

to pressure. The heat required to transform the disintegrated constituents of the compound to be produced may be derived from any external source of heat, or may 5 be produced by increasing the pressure to such a degree that the heat generated thereby incidentally produces the required state of plasticity.

Our novel process may also be applied 10 for the production of pressed bodies from a metallic element or other metallic substance and involves the considerable advantage of enabling one to produce the desired result in but one operation, whereas the 15 methods, as hitherto practised, require a repeated heating, mechanical treatment, and repressing of the metallic mass.

Instead of pressing the thus treated mass into an independent body of a desired shape 20 we may press the same upon another body and incidentally unite both to a composite body.

The term "reduced," as used in the specification and in the subjoined claims, indicates the procedure whereby a whole mass 25 of the substance is rendered less compact, which enables portions thereof to be readily separated from the main mass, and which permits the formation of an intimate mixture of the various substances.

It of course will be understood that the 30 illustrative embodiments of our invention above-described may be altered and varied within the scope of the subjoined claims.

35 We claim as our invention:

1. A process for the production of metallic bodies which comprises, reducing the primary metal, intermixing therewith a reduced substance, deoxidizing the primary 40 metal, heating the mixture until it becomes plastic, and subjecting the thus treated mass to pressure.

2. A process for the production of metallic bodies which comprises, reducing the primary metal, intermixing therewith a reduced substance, deoxidizing the primary 45 metal, covering said deoxidized mass with a protective layer of an inert gas to prevent reoxidation, heating the mixture until it becomes plastic, and subjecting the thus treated mass to pressure.

3. A process for the production of metallic bodies which comprises, reducing the primary metal, intermixing therewith a reduced substance, removing from the metallic 55 particles any film of oxide, heating the mixture until it becomes plastic, and subjecting the plastic mass to pressure.

4. A process for the production of metallic bodies which comprises, reducing the primary metal, intermixing therewith a reduced substance, treating the metallic particles with a mineral acid to remove any 60 oxide film, covering said deoxidized mass with a protective layer of an inert gas to

prevent reoxidation, heating the mixture until it becomes plastic, and subjecting the plastic mass to pressure.

5. A process for the production of metallic bodies which comprises, heating the 70 metal until it becomes plastic, deoxidizing said metal, and subjecting said deoxidized metal to pressure.

6. A process for the production of metallic bodies which comprises, heating the 75 metal until it becomes plastic, removing from said metal any oxide film, and subjecting said deoxidized metal to pressure.

7. A process for the production of metallic bodies which comprises, heating the 80 metal until it becomes plastic, deoxidizing said metal, covering the thus deoxidized metal with an atmosphere of an inert gas to prevent reoxidation, and subjecting said deoxidized metal to pressure.

8. A process for the production of metallic bodies which comprises, heating the metal until it becomes plastic, deoxidizing said metal, covering the thus deoxidized metal with an atmosphere of carbon dioxide 90 to prevent reoxidation, and subjecting said deoxidized metal to pressure.

9. A process for the production of metallic bodies which comprises, heating the primary metal until it becomes plastic, deoxidizing the said metal, intermixing said primary metal with another substance, and subjecting the mixture to pressure.

10. A process for the production of metallic bodies which comprises, heating the 100 primary metal until it becomes plastic, deoxidizing said metal, covering the thus deoxidized metal with an atmosphere of an inert gas to prevent reoxidation, intermixing another substance with said primary 105 metal, and subjecting the mixture to pressure.

11. A process for the production of metallic bodies which comprises, heating the primary metal until it becomes plastic, deoxidizing said metal, covering the thus deoxidized metal with an atmosphere of carbon dioxide to prevent reoxidation, intermixing another substance with said primary metal, and subjecting the mixture to pressure.

12. A process for the production of metallic bodies which comprises, fusing the metal, deoxidizing the fused metal, cooling the deoxidized mass down to a state of plasticity, and subjecting the plastic mass to pressure.

13. A process for the production of metallic bodies which comprises, fusing the metal, removing from the fused metal any 125 film of oxide, cooling the thus deoxidized mass down to a state of plasticity, and subjecting the plastic mass to pressure.

14. A process for the production of metallic bodies which comprises, fusing the 130

metal, deoxidizing the fused metal, covering the thus deoxidized mass with an atmosphere of an inert gas to prevent reoxidation, cooling the deoxidized mass down to a state of plasticity, and subjecting the plastic mass to pressure.

15. A process for the production of metallic bodies which comprises, fusing the primary metal, deoxidizing the fused metal, 10 cooling the deoxidized mass down to a state of plasticity, intermixing with said primary metal another substance, and subjecting the mixture to pressure while in the plastic state.

15 16. A process for the production of metallic bodies which comprises, fusing the pri-

mary metal, deoxidizing the fused metal, covering the thus deoxidized mass with an atmosphere of an inert gas to prevent reoxidation, cooling said deoxidized mass 20 down to a state of plasticity, intermixing with said primary metal another substance, and subjecting the mixture to pressure while in the plastic state.

In testimony whereof we have hereunto 25 set our hands in presence of two subscribing witnesses.

GEORG ISING.

HEINRICH BOROFSKI.

Witnesses:

WILHELM LEHRKE,  
WILLI FAHN.